

# UNITED STATES PATENT OFFICE.

JOHN H. RYAN, OF CHICAGO, ILLINOIS.

## PROCESS OF PREPARING PAPER-COATING COMPOSITION.

1,407,773.

No Drawing.

Specification of Letters Patent. Patented Feb. 28, 1922.  
Application filed May 6, 1920. Serial No. 379,315.

To all whom it may concern:

Be it known that I, JOHN H. RYAN, a citizen of the United States, residing at Chicago, county of Cook, and State of Illinois, have invented certain new and useful Improvements in Processes of Preparing Paper-Coating Composition, of which the following is a specification.

This application is a continuation in part 10 of my application for patent filed Sept. 22, 1919, Serial No. 325,467.

The invention relates to improved processes of preparing paper coating composition.

15 The object of the invention is to provide a superior coating composition of very fine texture and quality and at a reduced cost.

Objects relating to mere details will definitely appear from the detailed description.

20 In carrying out my improved process, I subject a quantity of clay or whiting, to the action of a pebble grinding mill. In case clay is being ground I mix the same with an equal quantity of water. Where whiting is being ground one half this volume of water is all that is required. This produces a thick creamy mixture or a mixture comparable to a thin dough. This is placed in a

25 pebble grinding mill, which is run at the usual rate so that the pebbles flow down over each other and through the mixture. They thereby grind all particles of grit to an imperceptible powder and, owing to their action upon the doughy mass, distribute the pulverized grit, which may be of a crystalline character throughout the colloidal mass in such a way that the crushed particles are separated and any possible reformation of

30 grit is obviated and also in such a way that no grit of considerable size can form anyhow.

When this is done I add sizing material, such as a proper solution of casein, glue or hydrated starch, and the mixture is further ground therein until a complete blend of the sizing has taken place with the thorough distribution of the minute grit that have been pulverizing. This last grinding consumes usually about one-half hour. The first period of grinding depends on the initial condition of the material and requires much longer.

Where casein is employed in the sizing

material, the necessary amount of alkaline compound, such as caustic soda, is added to insure its complete solution.

To the mixture above indicated may be added 50 parts of "satin white," the clay having been first prepared in the grinder as above outlined. The "satin white" and the casein may thus be added later. The mixture is then ground until all grit is pulverized and the particles distributed throughout the colloidal mass.

By following the methods above outlined, paper coating compounds may be prepared 65 of high grade quality and capable of producing papers also of high grade quality without the extensive screening of the mass heretofore found necessary.

I have thus described specifically the methods which I pursue, but desire to state that this method of treatment may also be applied to various coating compounds, the action of the pebble mill on the dough-like mass being to thoroughly pulverize any grit 75 and reduce the same to powder and distribute same through the colloidal mass induced by the action of the pebbles rolling through the heavy mass. This induces an action similar to that produced by the pulling of 80 candy in the manufacture of candy, and produces a comparable result, insuring great smoothness of the coating mixture.

In this behalf, I regard whiting as the substantial equivalent of clay, clay being the 85 broader description. Whiting requires only slightly different treatment.

Having thus described my invention, what I claim as new and desire to secure by Letters Patent, is:

1. The treatment of clay consisting in mixing the same with water until it is a thin doughy mixture, subjecting the same to the action of pebbles in a pebble grinding mill, adding the usual sizing solutions, and further grinding the same in a pebble mill to insure mixture and the pulverization and elimination of all grit, as specified.

2. The method of preparing coating composition which consists in first grinding a 100 mixture of water and a coating body, then adding sizing material including an alkaline compound, and further grinding the resulting mixture, substantially as described.

3. The treatment of coating composition 105

which consists in adding sufficient water to my hand and seal in the presence of two  
form a doughy paste, subjecting the material to the action of a pebble grinding mill  
to pulverize the grit therein and distribute  
5 the fine particles through the colloidal mass,  
as specified.

In witness whereof, I have hereunto set

witnesses.

JOHN H. RYAN. [L. S.]

Witnesses:

LUELLA G. GREENFIELD,  
MARGARET L. GLASGOW.